

## UNITED STATES PATENT OFFICE

FRANK R. PALMER, OF READING, PENNSYLVANIA, ASSIGNOR TO THE CARPENTER STEEL COMPANY, OF READING, PENNSYLVANIA, A CORPORATION OF NEW JERSEY

## FREE MACHINING CORROSION RESISTING STEEL

No Drawing.

Application filed December 7, 1929. Serial No. 412,576.

My invention consist particularly in a new and improved high chromium corrosion resisting steel having relatively free machining properties; corrosion, as herein used, comprehend attack by chemical reagents and oxidation or surface deterioration at elevated temperatures, and the corrosion resisting steels to which my invention relates being those in which the corrosion resistance has been imparted primarily by the element chromium.

Such steels are well known in the art, containing chromium from 2% to 60%, frequently modified by additions of copper, molybdenum, silicon, tungsten and nickel; the nickel element being often added in sufficient quantities to produce an austenitic non-magnetic steel, and the content aside from these elements being principally iron with sufficient carbon to accomplish the purpose desired in each case.

In my co-pending application No. 247,462 for an anti-friction and free machining corrosion resisting steel, I have fully pointed out how high chromium in steel renders the products difficult to machine, and how the deliberate employment of abnormally high percentages of sulphur overcomes the objectionable effect of the chromium without markedly interfering with the corrosion resisting properties. My present invention avoids some of the undesirable features of such high sulphur steel as specifically set forth in said earlier application; a main fact being that sulphur is objectionable from a merchandizing standpoint because it has been regarded for many years as a harmful ingredient, and that this prejudice is communicated to some extent to my high chromium corrosion resisting steels in which commonly prohibited high percentages of sulphur are deliberately employed. My present invention provides for producing a free machining product without incurring this objection incident to high sulphur content.

Furthermore, as pointed out in my prior application, the sulphur combines with various metals present in the steel to form metal-sulphides which are insoluble in the solidified steel, so that forged or rolled specimens

of high sulphur corrosion resisting steel, when polished and viewed under a metallurgical microscope, reveal considerable quantities of elongated slag-like sulphide inclusions which are objectionable in that they reduce the ductility and toughness of the metal in a direction normal to the direction of rolling or forging; whereas in my present invention, free machining qualities are imparted with decidedly less slag-like inclusions than in the case of high sulphur steels, constituting a very desirable improvement.

In the periodic table of chemical elements, sulphur occurs in a group having a valence of 2 with hydrogen and a valence of 6 with oxygen, usually referred to as group VI. This group is headed by oxygen which is a gas, and the elements of higher atomic weight than oxygen fall into two groups; one group comprising metalloids and the other group comprising metals. The metalloid group consists of sulphur, selenium and tellurium with atomic weights of approximately 32, 79 and 127 respectively. These three metalloids are known to be closely related in many of their properties and when referred to jointly hereinafter will be termed group VI metalloids.

I have found that selenium and tellurium have the property, when added to high chromium corrosion resisting steel, of imparting free machining properties in like manner to sulphur, and that they at the same time avoid the principal objections to sulphur above referred to. There is no general prejudice against selenium and tellurium, and their use therefore does not interfere with the merchandizing of the product; microscopic examination of a series of high chromium corrosion resisting steels containing various percentages of selenium and tellurium reveals that these metalloids, like sulphur, appear to combine with a metal, forming what is judged to be metal-selenides or metal-tellurides which appear very similar to metal-sulphides. However, the selenides and tellurides are evidently more soluble in the solidified steel than sulphides because a given percentage of either or both does not yield nearly so much slag-like inclusion as would the same percentage of sulphur. My examinations and tests

reveal no notable difference between the behavior of selenium and tellurium insofar as they are used to achieve the objects of this invention. They apparently can be variedly used with ordinary judgment, either individually, or jointly, and with or without sulphur, so as to satisfactorily achieve the stated results aimed for.

I have further discovered that it is not necessary to use as much selenium or tellurium, singly or jointly, as would be necessary in the case of sulphur alone to secure satisfactory machining properties. As pointed out in said application, No. 247,462 sulphur has little effect on the machining properties of high chromium corrosion resisting steel, particularly when the chromium exceeds 10.00%, until the sulphur exceeds .15% by weight of the mass; whereas I have obtained very satisfactory machining properties by using only about .07% of selenium or tellurium, though I have found the optimum percentage of these new metalloids to be about .20% by weight. So far as I am aware neither selenium nor tellurium have been heretofore used in any ferrous alloy for the present stated purpose, or any other.

High chromium corrosion resisting steels, as now commonly employed, contain about .20 to .50% manganese. In my prior application No. 247,462, I have pointed out that hot malleability may be preserved in high sulphur corrosion resisting steels by increasing the manganese percentage above this normal range or by the addition of a metal like zirconium, in order to prevent the formation of a preponderance of iron-sulphide with resultant red shortness. In my present invention, since tellurium and selenium, singly or jointly, need not be added in such large percentages as sulphur, and also presumably because of their partial solubility in the steel base, the need for special alloy additions to secure hot malleability is not so vital. Nevertheless, I prefer, in the interests of good steel making practice, to use increased manganese or a metal like zirconium in conjunction with the metalloids noted.

My invention is fully embodied in high chromium corrosion resisting steels of the following type compositions:

|     | Carbon | Chromium | Sulphur | Zirconium | Selenium | Tellurium |
|-----|--------|----------|---------|-----------|----------|-----------|
| (a) | .10    | 14.00    | .02     | .15       | .20      | —         |
| (b) | .10    | 14.00    | .02     | .15       | —        | .20       |

I have carefully compared steels of the above type compositions with steels of the following type compositions:

|     | Carbon | Chromium | Sulphur | Zirconium | Selenium | Tellurium |
|-----|--------|----------|---------|-----------|----------|-----------|
| (c) | .10    | 14.00    | .02     | .15       | —        | —         |
| (d) | .10    | 14.00    | .02     | .15       | —        | —         |
| (e) | .10    | 14.00    | .30     | .15       | —        | —         |

Steels (c) and (d) do not machine satisfactorily with the usual machine shop practice because the chips tend to gall and adhere to the tools, producing a condition frequent-

ly termed "gummy machining". Steels of the analysis of (a), (b), and (e) machine with approximately equal facility and can be cut with standard shop tools at high speeds with relatively little galling of the chips and with a good smooth finish.

My invention applies with proportionately the same effectiveness to high chromium corrosion resisting steels containing minor percentages of other alloys such as silicon, copper, molybdenum and tungsten; and with nickel additions even sufficient to produce an austenitic product, the application of my invention produces marked improvement in machining properties.

Steels within the scope of this invention can readily be made in a crucible pot furnace by compounding the corrosion resisting base analysis steel in accordance with usual crucible steel melting practice and adding metallic selenium or tellurium or both, just before pouring the metal from the crucible. Both metalloids are quite volatile and should be added in stick form rather than as a powder, and losses can be reduced by thrusting the metalloids beneath the surface of the molten steel on the end of a rod. In any case an excess of metalloid ranging from 2 to 10 times the residual quantity required should be allowed for volatilization, the exact excess necessary varying according to the individual melter's manipulations in adding the metalloids. These improved free machining steels can also be made in the electric furnace but the selenium and tellurium should be added in the ladle with due provision for loss.

It is to be understood from the above description, that my present invention is a further development of the invention specifically set forth in my said prior application Serial No. 247,462, it being based on determination of the fact that the elements selenium and tellurium, of the recognized periodic group VI, may be used individually or jointly to replace wholly or in part the sulphur of said group, and with stated advantages over use of sulphur alone as previously described; the essential desired effect of free machining being apparently always secured, with and incidental to resulting reduction of high frictional quality in the alloy; and such main desired effect being secured by an actual content in the alloy of between .03% and 2.00%, of the group VI metalloids.

What I claim is:

1. As a composition of matter an alloy steel containing chromium between 4% and 60% and the elements selenium and tellurium of a total percentage between .03% and 2%, and characterized by relatively free machining quality.

2. As a composition of matter, an alloy steel containing chromium between 4% and 60% and selenium between .03% and 2%, and

characterized by relatively free machining quality.

3. As a composition of matter an alloy steel containing chromium between 4% and 60% and tellurium between .03% and 2%, and characterized by relatively free machining quality.

In testimony whereof I affix my signature.

FRANK R. PALMER.

10

15

20

25

30

35

40

45

50

55

60

65